

July 2, 1946.

P. E. JAMES

2,403,084

APPLICATION OF MARKINGS TO SURFACES

Filed Jan. 28, 1942

Fig. 1.



Fig. 3.



Fig. 2.



Fig. 4.



Fig. 5.



Fig. 6.



WITNESSES:

Robert C. Baird  
Frederick Shaper

INVENTOR

Paul E. James.  
BY  
Gra. W. Savage  
ATTORNEY

## UNITED STATES PATENT OFFICE

2,403,084

## APPLICATION OF MARKINGS TO SURFACES

Paul E. James, Mansfield, Ohio, assignor to Westinghouse Electric Corporation, East Pittsburgh, Pa., a corporation of Pennsylvania

Application January 28, 1942, Serial No. 428,492

4 Claims. (Cl. 41—26)

1

This invention relates to the application of markings, such as indicia, legends and ornamentation, to the surfaces of members, more particularly in combination with painted surfaces. The markings may be applied in the process of applying colored protective finishes to members and form an integral part of the protective finish.

Heretofore whenever indicia, legends or ornamentation have been applied to the painted surfaces of members, it has been necessary, as a rule, to apply the appropriate markings by superimposing them on the organic finish comprising the painted surface. Markings so produced were subjected to rapid wearing away due to their surface position. Even the normal cleansing of the member bearing the markings resulted in a disproportionate deterioration and removal of the substance comprising the marking with the consequent blurring and illegibility. The applied markings consequently were rapidly scratched, abraded and washed off, so that they quickly became faint and shabby in appearance.

The object of this invention is to provide for marking painted surfaces by applying coloring material as an integral part of the paint on the surfaces.

Another object of the invention is to provide for so applying coloring material as markings to predetermined areas of a painted surface of a different color that the surface may be repainted with the applied coloring material penetrated through the repainted surface.

Other objects will, in part, be obvious and will, in part, appear hereinafter in the specification and claims.

For a more complete understanding of the nature and objects of the invention, reference should be had to the following drawing, in which:

Figure 1 is an elevational view of a prior art type of marking on a painted surface;

Fig. 2 is a section of Fig. 1 on line II—II;

Fig. 3 is an elevational view of the invention applied to a member;

Fig. 4 is a sectional view on Fig. 3 of line IV—IV;

Fig. 5 is a view showing the consecutive steps for producing the markings according to the invention;

Fig. 6 is a section of Fig. 5 on the line VI—VI;

Fig. 7 shows a modified embodiment of the invention;

Fig. 8 is a section of Fig. 7 on the line VIII—VIII; and

Fig. 9 shows the invention applied to a refrigerator.

2

Numerous commercial articles from metals, wood, fibrous materials of all types and similar materials of construction are completed in manufacture at the present time by the application of a protective organic finish to the surface of the material after the processing of the material to final shape has been substantially completed. Organic finishes so applied have the general function of protecting the underlying material from corrosion, rusting, rotting or deterioration, as well as providing for a body color and for decorative appearance. In addition to a general application of organic finish for such purposes, it is customary to apply thereover ornamentation comprising applications of a differently colored finish in the form of stripes, borders, and numerous other configurations. In some cases, trade-names and trade-marks are applied by superimposing appropriate substances over the protective organic finish in order to acquaint the trade with the source and type of product. In some cases, legends describing modes of operation and precautions to be exercised in handling the device are also applied in this manner. Furthermore, name-plates and equivalent data, including serial number, model number, date of manufacture and other pertinent information may be applied to apparatus by means of paint applied through stencils or stamps to the exterior surface of the protective organic finish.

The application of legends, indicia and ornamentation to a general painted coating or protective organic finish, such as described, and their equivalent will be designated hereinafter as "markings." As a rule, the markings are not intended to contribute materially to the protection of the surfaces underlying the protective organic finish, but are simply applied for decorative or informative purposes.

40 Markings applied to the exterior surface of the painted members are most effective if they retain their configuration and do not fade or otherwise deteriorate any more rapidly than the body of the paint. However, due to the relatively raised 45 and exposed position in which the markings are applied, they are subjected to more wear than the main body of the protective organic finish. In cleaning the members, for example, the edges of the markings are subjected to considerable 50 wear due to the fact that the markings stand above the surface of the organic finish. The cleansing tool or implement tends to abrade the exposed markings much more rapidly than the 55 remainder of the organic finish. Ordinary wear

and tear also causes a disproportionate fading and loss of the markings as heretofore applied.

According to this invention, markings are applied to painted surfaces or, more generally, to protective organic finishes upon surfaces of members as an integral part of the protective organic finish. Therefore, the markings, while standing out visually from the remainder of the painted surface, are substantially an integral part of the same smooth painted surface and are subjected to wear and tear in the same proportion as the remainder of the organic finish. In addition, the markings are applied so rapidly and simply by means of the invention to be disclosed that it constitutes a matter of great economy to apply markings by the process of the invention. The markings may be applied as any contrasting color in combination with a protective organic finish of any type, form or color. Other advantages of the invention will be outlined hereinafter.

As an example of the prior art practice of applying markings, reference should be had to Fig. 1 showing a member 10 carrying such applied marking. The member 10 comprises a body 12 of suitable material and a protective organic finish coating 14 upon its surface. The protective coating 14 may include primer coatings and subsequent finish coatings in any combination. The protective coating 14 has a surface which is finished in the desired color and with predetermined smoothness and gloss. It is a completely finished article except for the marking 16 which is subsequently applied thereto. In the example of Fig. 1, the marking 16 comprises an indicia composed of the letter "W." The indicia has been applied, for example, by means of a perforated stencil and a layer of organic finish deposited through the stencil perforation upon the protected coating 14. In other cases, the indicia 16 has been a decalcomania which has been adhesively applied to the coating 14. In any event, it will be noticed by reference to Fig. 2 that the main body of the indicia 16 is elevated above the surface of coating 14 and is, therefore, subject to be abraded and worn prematurely, as mentioned herein, which, in some cases, may reflect upon the quality of the manufacture of the device.

This invention has for its object the application of markings as a part of a general application of protective organic finish to any given member. It has been discovered that organic dyes which are soluble in one of the constituents of the protective organic finish may be so applied in combination with the organic finish that the dye produces markings integral with the organic finish.

Reference should be had to Figs. 3 and 4 of the drawing showing one form of the application of the invention. The member 12 carries a protective coating 14 applied to one entire surface. The coating carries as an integral part thereof an organic dye in the form of the indicia 18 comprising a "W." By reference to Fig. 4, it will be noticed that the indicia 18 is not upraised above the level of the coating 14, but extends substantially entirely through the thickness of the coating 14 to the base member 12, and is substantially of the same thickness. In this case, the indicia will exist as long as coating 14 while functioning to give any desired visual impression.

The terms "painted surface" and "protective organic finish" are intended to include the application of all types of protective substances having an organic base applied to surfaces. This includes finishes or paints generally composed of

resinous film-forming materials and solvents and additions to the film-forming materials, the solvents including high boiling-point materials which may serve as plasticizers or in other functions, and low boiling-point solvents to thin the finish to facilitate application to surfaces and subsequently rapidly evaporating from the film-forming resins to produce an effective protective coating. The protective finish need not contain added pigments or other coloring material, but the invention will function as satisfactorily if pigments or other coloring matter are added to produce any predetermined color of painted surface. It is intended to include synthetic resin lacquers, enamels, varnishes and other commonly employed finishes in the scope of this invention.

The invention consists of the application, in combination with the protective finishes, of organic dyes characterized by solubility in a solvent which is employed in the organic finish. For instance, in combination with nitro-cellulose lacquers and enamels containing polar type solvents, various aniline dyes have been quite successfully employed as marking materials. Aniline blue, fuchsin and malachite green are examples of some of the successfully applied organic aniline dyes. Other dyes soluble in polar type solvents such as methylene violet, nigrosin, Congo red, indigo carmine, and eosin also have been used with satisfactory results. Oil soluble dyes such as Sudan III and azolitmin have functioned with nitrocellulose base finishes to produce excellent results. All of the dyes listed have been employed equally successfully in combination with urea-formaldehyde type of lacquers. Glycerol phthalate lacquers also have been associated with the same dyes to produce successful markings. In some cases, Melamine enamels have been combined with the organic dye and subjected to high temperature baking with the markings resulting being of the highest degree of legibility and clearness. Other lacquers have been both air-dried and baked with applied organic dye markings with satisfactory results.

For a mode of application of the invention, reference should be made to Figs. 5 and 6. The member 20 composed of steel, for example, is coated with a primer 22 which may be conveniently an oil base metal primer which is conventionally baked for a short period of time. In the next step of the process, the organic dye 24, dissolved in a suitable solvent as will be more specifically disclosed hereinafter, is applied in predetermined configuration corresponding to the marking desired on the primer coating 22 on the member 20. The organic dye generally impregnates and penetrates through the primer to the member 20. Thereafter, the member is treated by spraying the normal finish coating 28 over the primer coating. The finish coating, for example, in many household appliances consists of a heavily pigmented nitro-cellulose enamel or a urea-formaldehyde enamel. The finish coating having been applied, the member 20 is baked for a period of about one hour at a suitable temperature.

When the member 20 is removed from the oven, it will be discovered that organic dye has completely penetrated through the finish coating to produce a clear and legible indicia 26. The dye 26 is substantially distributed throughout the entire thickness of both finish coat and primer coat. On testing the surface by abrading with an abrasive cleaning compound, it will be discovered that

both the indicia and the finish coat are equally and uniformly removed.

In case aniline dyes or other water soluble dyes have been used, it has been discovered that the application procedure shown in Figs. 5 and 6 produces an indicia which is not water removable. Panels so prepared have been subjected to running water for many hours without any noticeable washing out of the dye. In humidity tests conducted at 100% humidity and running for hundreds of hours no bleeding of the dye or washing has occurred, even though the surface of the member will continuously carry a film of moisture during the test. In the case of non-polar dyes such as Sudan III, the marking applied in this manner has withstood all tests conducted at high humidities at low and high temperature, and exposure to light, and other deteriorating influences without any appreciable fading or other undesirable result.

It is not necessary that the organic dye be applied on the primer coat of the material, though this has been found to comprise the most practical and economical method of applying organic dye markings to members carrying a protective finish. The organic dye may be applied to the bare metal surface or bare metal surface carrying a phosphate or other rust-inhibiting coating. Thereafter, the primer and the coats of organic finish may be applied with the dye penetrating through the thickness thereof to the exposed surface. It will be found that the dye will be relatively uniformly dispersed through the organic finish. It should be mentioned here that dye marking does not tend to smudge or tend to spread irregularly laterally.

In some cases, where the finish coat has already been applied to a member, markings may be produced by applying the dye to the external surface thereof with certain subsequent treatment to protect the dye. Aniline dyes have been applied to the external surface of the paint, and it is found that the dyes will penetrate into the painted surface. It will be appreciated, however, that since water soluble dyes so applied may tend to smudge slightly when a moist rag is run over the surface due to the high concentration there, it is desirable to apply a sealing film of transparent lacquer or even pigmented enamel thereover.

Referring to Figs. 7 and 8 of the drawing, there is illustrated the product resulting from this latter mode of applying markings. The steel base member 20 carries a primer coating 22 and finish coating 28 of protective finish. The organic dye 44 has penetrated into both layers 22 and 28 as well as into the subsequently applied sealing coating 42 which is shown as a contrasting color area. The sealing coating 42 serves to maintain the effectiveness of the dye 44. This method may be used on articles already painted when purchased. Thus painted delivery trucks may be marked by the purchaser with the owner's name and business, with a final sealing coat of transparent lacquer applied over the markings.

In applying the dye to the organic finish, it has been discovered that the dyes, which generally are solids or powders, are best applied in a solvent or liquid carrier. Rapid drying solvents are not as convenient carriers for the dye as compared with slower evaporating liquid carriers. It has been found that the dye may be applied with highly satisfactory results if the dye is dissolved in a transparent or clear organic finish of the same type as the finish coating on the member.

For example, if a nitro-cellulose base lacquer is to be applied as the finish coating on a member, an aniline base dye, such as indigo carmine, may be dissolved in transparent nitro-cellulose base lacquer and applied to the primer coating. Equal parts by weight of dye and transparent lacquer are suitable proportions. Shellac, that is the ethyl alcohol solution of lac, may be used as the liquid carrier for the dye. In other cases, a special type of carrier may be prepared for the dye. Polar type dyes may be dissolved in a mixture of an alcohol plus a high boiling point liquid, such as diethyl phthalate. A mixture so prepared does not dry out as rapidly as ethyl alcohol, therefore the dye may be applied more effectively. Generally the dye is present in the carrier in larger amounts than is ordinarily present in ordinary finishes.

The dye solution prepared as indicated may be applied to members by any one of numerous means. The organic dye, for example, may be applied by means of a stamp pad and stamp using the pad saturated with the dye in a slow evaporating solvent. In other cases, the dye may be applied by means of a stencil with openings provided for the suitable marking with the dye either being sprayed on or brushed through. In some cases, for example, in applying striping to appliances or automobile bodies, the dye may be applied by means of a brush or roller applicator or a spray gun having a suitably adjusted spray. Several dyes may be applied adjacent one another. Other methods of application of the dyes in predetermined coloring form and amount will be readily evident.

The combination of organic finish and dye to produce predetermined markings has been applied to glass, phenol formaldehyde moldings, polystyrene molding, acetabutylate moldings, cellulose acetate moldings, and other plastics, as well as wood and steel. The organic dye has been applied in combination with many protective finishes. White finishes, gray finishes, and black finishes have been marked with great success by employing contrasting color dyes.

As an example of the finished product, reference should be made to Fig. 9, showing a commercial type of refrigerator 30. The refrigerator comprises a door 32 painted a glossy white which carries as markings, three vertical stripes 34, 36 and 38, and a trade name plate 40. The overall surface of the door 32 is composed of a pigmented, white urea-formaldehyde type of organic finish. The stripes 34, 36 and 38 may consist of an organic dye, for example, Sudan III applied as an integral part thereof. The name plate 40 is composed of an aniline blue dye applied as an integral part thereof according to the procedure shown in Figs. 5 and 6.

Previously, decalcomanias had been used for the trade-mark 40 and had been found to be so lacking in sufficient life with attractive appearance that it was necessary to emboss or indent the panel 32 to provide a protective depression for the decalcomania. By means of this invention, this operation on the door has been eliminated.

In a household appliance such as the refrigerator shown in Fig. 9, it is customary to apply to the back thereof certain indicia indicating the model number, serial number, and other desirable information. It has been found that when a dye is applied in the manner disclosed herein to the back of the refrigerator, particularly if a nitro-cellulose base liquid is applied as a finishing coating, though not limited to this lacquer, that

the surface may be repainted with subsequent applications of nitro-cellulose lacquer and the indicia will penetrate through the subsequent lacquer coatings and be legible. As many as three successive repaintings have been applied over indicia of this type and the indicia have been perfectly transparent and legible after each repainting job. There is a slight diminution of the intensity of the dye with each repainting so that the markings become less clear, and it would not be desirable to repaint, for example, five or six times. For most practical purposes, ability to undergo two or three repaintings is sufficient.

Heretofore, when refrigerators have been repaired, occasionally the backs have been repainted, thereby covering up the information carried thereon. However, by means of the present invention, such repainting does not affect the indicia and the information is just as legible after repainting as before. Since no other information application known is capable of functioning to withstand repainting and still show up in contrasting colors, the present invention presents a decided advantage.

Since certain obvious changes may be made in the above processes, and different embodiments of the invention could be made without departing from the scope thereof, it is intended that all material contained in the above description or taken in connection with the accompanying drawing shall be interpreted as illustrative and not in a limiting sense.

I claim as my invention:

1. An article of manufacture comprising a member, a protective coating of a substantially uniform thickness applied to the surface of the member, the protective coating composed of a primer coating and a finish coating, the finish coating having a given color and including organic resins, and predetermined areas of the coating having a different color to provide for markings, the different color comprising an organic dye applied to the primer coating and extending substantially through the entire thickness of primer and finish coatings, the finish

45

coating lessening deterioration of the applied organic dye markings.

2. An article of manufacture comprising, a member, a protective coating applied to a surface of the member, the protective coating being of substantially uniform thickness and including a primer coating and a finish coating, the finish coating composed of organic resins and having a given color, predetermined areas of the protective coating being of a different color than said given color, the different color composed of an organic dye applied to the finish coating and penetrating through substantially the entire thickness of the protective coating, and a sealing coating applied to the predetermined areas to lessen deterioration of the organic dye, the organic dye extending through the thickness of the sealing coating.

3. The method of applying markings to a member having a surface painted with a coating composition having a given color, comprising applying to the member an organic dye soluble in a solvent employed in the coating composition, the organic dye being so applied as to produce the markings desired, applying the coating composition paint upon the base member over the applied dye, whereby the dye penetrates the thickness of the applied coating composition and is visible at the surface, and drying the painted surface.

4. The method of producing an article with a painted surface carrying colored markings, comprising applying a primer coating material to the article, drying the primer coat, applying an organic dye to the dry primer coat in a configuration corresponding to the desired colored markings, applying a finish coating to the article, the finish coating including film forming resins and a solvent for the resins capable of dissolving the organic dye whereby the dye penetrates both into the primer coats and through the finish coating, and treating the finish coating to dry and harden the coating.

PAUL E. JAMES.